

July 26, 1938.

C. P. BRATASIANU

2,124,905

PROCESS FOR MANUFACTURING CAST IRON AND OTHER MATERIALS

Filed June 11, 1934

5 Sheets-Sheet 1

Fig. 1.



Inventor:  
C.P. Bratasianu,

by E.F. Stendroth  
Atty.

July 26, 1938.

C. P. BRATASIANU

2,124,905

PROCESS FOR MANUFACTURING CAST IRON AND OTHER MATERIALS

Filed June 11, 1934

5 Sheets-Sheet 2



Inventor:  
C. P. Bratasianu,

By G. F. Mandroth  
Att'y.

July 26, 1938.

C. P. BRATASIANU

2,124,905

PROCESS FOR MANUFACTURING CAST IRON AND OTHER MATERIALS

Filed June 11, 1934

5 Sheets-Sheet 3

Fig. 3.



Fig. 6.

Inventor:  
C. P. Bratasianu,

by G. F. Kunderth  
atty.

July 26, 1938.

C. P. BRATASIANU

**2,124,905**

## PROCESS FOR MANUFACTURING CAST IRON AND OTHER MATERIALS

Filed June 11, 1934

5 Sheets-Sheet 4

Fig. 4.



Fig. 7.



Inventor:  
C.P.Bratasianu,  
by G. F. Wunderth  
Alt'y.

July 26, 1938.

C. P. BRATASIANU

2,124,905

PROCESS FOR MANUFACTURING CAST IRON AND OTHER MATERIALS

Filed June 11, 1934

5 Sheets-Sheet 5

Fig. 5.



Fig. 8.



Inventor:  
C. P. Bratasianu,

by A. T. Hendrik  
Atty.

## UNITED STATES PATENT OFFICE

2,124,905

PROCESS FOR MANUFACTURING CAST IRON  
AND OTHER MATERIALS

Constantin Paul Bratasianu, Craiova, Rumania

Application June 11, 1934, Serial No. 730,081  
In Rumania June 13, 1933

9 Claims. (Cl. 75—40)

This invention relates to a process for treating simultaneously and together, by chemical and metallurgical means, solid combustible materials of poor quality to improve them, heavy hydrocarbons to convert them into light hydrocarbons, and iron ores to carburize them, and for then treating these improved products in a metallurgical furnace for the purpose of obtaining synthetic cast iron, that is to say cast iron having a low and controllable carbon content or special steels ultimately rich in manganese, aluminium, silicon, etc. in a single fusion operation.

It is known that iron ores are treated in blast-furnaces to obtain cast iron and that the respective steps consist in heating the ores in contact with metallurgical coke or wood charcoal and fluxes; and in injecting hot air, and that the pigs thus obtained are later converted by other metallurgical operations into steels.

It is also known that heavy hydrocarbons of poor quality such as the residues of the distillation of petroleum-bearing products (mazout) or of tars, are converted into light hydrocarbons having a low boiling point by depolymerization or by cracking by processes consisting in heating them at temperatures and pressures frequently of a very high order, and sometimes in the presence of catalysts. The known processes have the disadvantages, however, that the light products produced often contain phenols, that their yield is reduced, and that they produce large quantities of coke of poor quality or of minimum value.

It is known, moreover, that a coke of high value, that is to say, a metallurgical coke, can only be obtained from a combustible material of good quality which contains only a certain definite amount of gas, no sulphur, and only a little mineral material which is converted into ash.

The process according to the present invention provides the possibility of manufacturing cast iron or steel directly in two chemical and metallurgical operations, which are carried out in several stages in a series of suitable apparatus, starting with poor pulverulent ores, even containing sulphur, combustible materials which have up to the present not been convertible into coke, and heavy hydrocarbons such as the residues from the distillation of raw petroleum or from distillation of other combustible materials. It will be understood that the process may be varied to suit varying circumstances or requirements, either as to the amount, or the properties of one or other of the products, and that it may

be interrupted after one or other of the stages, taking an intermediate product as a final product, such as metallurgical coke or a light hydrocarbon capable of use in internal combustion engines or a purified, enriched or carburized ore. The total amount of solid materials present is not less than half that of the liquid hydrocarbons.

In accordance with the principal feature of the invention the process for the production of improved cast iron, or steel, and/or for the production of improved intermediate products is characterized by the fact that firstly, iron ores, solid carbonaceous and distillable combustible materials and heavy hydrocarbons (which may all be of poor quality) are subjected to heat treatment at a relatively low temperature (of the order of 500° C.), whereby there are produced high quality metallurgical coke, light hydrocarbons, and purified and carburized ore, and, secondly, said intermediate products (high quality coke, hydrocarbons and ore), so produced, are, if desired, subjected to heat treatment in a fusion furnace at relatively high temperature (of the order of 2000° C.) with the addition, if required, of fluxing materials, whereby there are produced in a single fusion operation, synthetic pig iron or special steels.

Also in accordance with the invention a special furnace, hereinafter fully described, is used for carrying out said process. The invention is also concerned with the improved products produced by the said process.

To carry out the process, there may be used:

A solid, poor quality combustible material, such as wood, lignite, coal non-convertible into coke, and even containing sulphur.

An iron ore, fragmentary or pulverized, containing oxides of iron, manganese, chromium, silicon ( $MnO$ ,  $MnO_2$ ,  $SiO_2$ ) and even an ore containing sulphur.

A residue from the distillation of petroleum, even a paraffinous residue, or a tar.

All these starting materials, taken in proportional amounts depending on their characteristics, and those of the products to be produced, are introduced together at atmospheric pressure in a retort subject to heating from outside. It is to be noted that the first operation is to be carried out at a relatively low temperature, about 500° C., and that the iron oxide and the ores which take part in the reaction serve simultaneously as catalysts, which is the reason why the reactions can be effected at such low temperature.

The interactions which take place simultaneously between the starting materials and between the products of their distillation or their cracking during the operation, these products being in a nascent condition and in the presence of a catalyst, are very complex and cannot yet be fully explained, but having regard to the practical results achieved, it is thought that they are, shortly, as follows:—

10 (a) the water contained in the combustible material and the ore is dissociated to produce oxygen (O) and hydrogen (H);  
 (b) the combustible material distils, and gives off tars, hydrogen (H) and methane (CH<sub>4</sub>), whilst a part of its carbon combines with a part of the oxygen obtained under (a) to form carbon monoxide (C+O=CO);  
 (c) the ore, upon contact with the carbon monoxide formed under (b) is subjected to reduction and carburization giving rise to the formation of carbon dioxide (FeO+CO=CO<sub>2</sub>+Fe) which, by a reversible reaction, combines with the carbon of the combustible material (CO<sub>2</sub>+C=2CO), whilst the ore is carburized on contact with the free carbon set free in the mineral; on the other hand, the catalytic action of the carbon monoxide in the presence of water vapour gives rise to the formation of hydrogen

20

25

30



which serves, in conjunction with the hydrogen resulting from the dissociation of the water under (a), to hydrogenize the distillation products of the hydrocarbons or tars introduced into the reaction;

35 (d) the hydrocarbons (residues or tars) introduced commence by being decarburized by the available oxygen arising from the water vapour given up by the ore and combustible material, and by becoming hydrogenized at the same time by undergoing polymerization or cracking in the medium rich in hydrogen. It is here that isoparaffins and olefines are formed, and the formation of phenols avoided, as the distillation takes place in a medium rich in hydrogen and in methyl (CH<sub>3</sub>) which arise either from the combustible material or from the methane under (b) or even from the synthesis of the hydrocarbons created, according as they are depolymerized.

40 50 The sulphur content of the combustible material or the ores is removed from the reaction by the following reactions:



From this there results either a gas, or colloidal sulphur which passes into the waste (pitch, ashes, etc.).

60 This first operation of the process thus gives:

65 1. Metallurgical coke, i. e. an enriched combustible material obtained from a poorer quality combustible, which may even be pulverized, the calorific power of which is increased by the carbon from the conversion of the residue or of the tars, which carbon is at the same time a binder.  
 2. Ore already agglomerated and carburized, without commencing to melt, in the same manner as the combustible material, which ore being already carburized, that is to say, already containing carbon, can be more easily cast than the ore which is usually introduced into the blast furnace and where it was first carburized by contact with the incandescent coke.

70

75

3. Light hydrocarbons rich in aromatics, which arise from the tars, and also in isoparaffins and olefines.

The next step of the present process is carried out in the fusion furnace described below, into which the products already obtained (i. e. the coke, the ore, and the hydrocarbons in the proportions necessary to obtain the desired result) are introduced.

Example

10

To carry out the first operation of the process there were used:—

150 kilograms of residues from the distillation of 15 petrol (mazout).  
 50 kilograms of pulverized iron ore containing manganese and a little sulphur.  
 100 kilograms of wood having a calorific power of 2500 to 3000 calories per kilogram. 20

The yield was as follows:—

- (a) 45 kilograms of carburized ore, agglomerated and sulphur-free;  
 (b) 48 kilograms of agglomerated metallurgical coke having a calorific power of about 8000 calories per kilogram;  
 (c) 150 kilograms of light hydrocarbons, which when submitted to official analyses showed that: 30

the fraction of this hydrocarbon which distils up to 95° C. is 34.07% and up to 200° C. is 89.5% of the total amount; the fractions which distil up to 150° C. contain no phenol, those which distil between 150 and 200° C. contain 1.76% of phenols and the heavier fractions contain 3.10% of phenol. 35

There are thus obtained from 100 kilograms of solid combustible material having 2500 to 3000 calories per kilogram, 48 kilograms (i. e. 48%) of metallurgical coke having 8000 calories per kilogram, this being a combustible product of which the total calorific content is greater than that of the starting material, whilst with other processes there would have been obtained approximately only 30% of wood charcoal having 7000 calories per kilogram. 40

It is to be pointed out that in other similar experiments carried out in accordance with this process, with lignite, of which the calorific power was about 3500 calories per kilogram there was obtained a quantity of 60-70% of metallurgical coke having 7700 calories per kilogram and sulphur-free. 45

50 55 Since the results of experiments (including amongst them the example given) prove that the total amount of coke obtained contains more calories than the amount of wood introduced, it must be admitted that this result can only be attributed to the fact that the derived products rich in aliphatic carbon, in the form of vapour, resulting from the heavy hydrocarbons introduced in the reaction become attached to the combustible material by an action similar to cementation or by a reciprocal penetration which takes place between the solid combustible material (which distils) and the heavy hydrocarbons which undergo dissociation. The combustible material which distils, is first freed of the light 60 gases such as hydrogen (H) and methane (CH<sub>4</sub>) which diffuse amongst the heavy hydrocarbons, whilst the aliphatic carbon which results from the conversion penetrates in the form of carbon monoxide (CO) into the combustible material, 65 70 75

where it becomes converted in accordance with the equation



this latter carbon becoming attached to the combustible material. This reaction continues until the combustible itself commences to give off tars which, on contact with the dissociation products of the hydrocarbons, become agglutinants and penetrate afresh into the combustible material and effect its agglomeration.

Next, it is seen that from 150 kilograms of heavy hydrocarbons introduced into the reaction, there result 89.5% of light hydrocarbons capable of use in internal combustion engines, and it is to be noted that by controlling the reaction judiciously almost 100% may be obtained.

The results of experiment thus show another particular advantage of the new process, namely, that the distillation products arising from carbonization at low temperature of carboniferous materials become mixed, immediately they are formed, with the hydrocarbons which have been introduced, and it is in combination with the latter that they are submitted to cracking, in such a way that the yield of light products is greater than would be obtained by submitting to the cracking operation only the hydrocarbons introduced.

The result of experiment shows, as in the example given, that the process according to the invention gives, by the conversion of heavy hydrocarbons, other light ones, which distil between 150 and 200° C. and which are free from phenol, whilst the light hydrocarbons obtained by other processes contain up to 40-50% of phenol. In the new process the essential fact is that the tars from the solid carbonaceous material and the heavy liquid hydrocarbons undergo cracking together in the presence of hydrogen. This hydrogen results from the dissociation of water vapour, which water was contained in the solid combustible and the ore, and hydrogen from the reactions themselves as is evolved during the distillation in the presence of catalysts. These catalysts are the ore (preferably rich in manganese, such as MnO and MnO<sub>2</sub>), the carbon (C) and the carbon monoxide (CO), which in a medium rich in hydrogen gives rise to reactions which free the water and methane



On the other hand the distillation of the solid carbonaceous material gives rise to methyl alcohol (CH<sub>3</sub>OH). Due to the catalysts the hydroxyl (OH) is broken away and having the methyl radicle (CH<sub>3</sub>) which prevents the formation of phenol and which, being unstable, combines to form ethane in accordance with the equation CH<sub>3</sub> + CH<sub>3</sub> = C<sub>2</sub>H<sub>6</sub>, which latter, losing successively its hydrogen, changes to ethylene (C<sub>2</sub>H<sub>4</sub>) and finally acetylene (C<sub>2</sub>H<sub>2</sub>), which by polymerization changes to benzene (C<sub>6</sub>H<sub>6</sub>). Thus by synthesis an entire light hydrocarbon series is obtained capable of being used in all types of motors.

The enriched products obtained in the first operation of the process (i. e. the carburized agglomerated sulphur-free ore, the metallurgical coke, also sulphur-free, as well as the light hydrocarbons free from sulphur, phenols or other oxygen compounds—if it is not intended to use them as such—are then treated in a second operation for the finishing of the process, that is, for making in a single fusion operation synthetic pigs or special steels. To this end the enriched

products are introduced into a suitable furnace, preferably into the special furnace which is one feature of the invention and which is described hereinafter. Besides these products there are introduced fluxes, additions of ores rich in manganese to regulate oxidation and to eliminate eventual traces of sulphur in the combustible material or the ore. There may also be added iron waste or scrap.

This special furnace is a shaft furnace the total height of which need not exceed 7 to 8 metres. It has a lining which, at the high temperature at which it works (about 2000° C.) produces slag similar to cement, from which flagstones, tiles, etc. may be made.

One embodiment of the furnace referred to is shown by way of example in the attached drawings, in which:

Fig. 1 is a vertical longitudinal section through the furnace and its accessory fittings;

Fig. 2 is a horizontal section along line 2—2 of Fig. 1, also of the furnace and its accessory fittings;

Fig. 3 is a vertical transverse section along line 3—3 of Fig. 2 of the whole installation;

Fig. 4 is a section similar to that of Fig. 3 but showing the furnace proper to a greater scale;

Fig. 5 is a section similar to that of Fig. 1, showing the furnace alone to a greater scale;

Fig. 6 is a section similar to that of Fig. 2 showing only the absorption chamber of the furnace to a greater scale;

Fig. 7 is a horizontal section along line 7—7 in Fig. 5;

Fig. 8 is a horizontal section along line 8—8 in Fig. 5.

The furnace functions at very high temperature reaching near 2000° C. produced by the injection of the hydrocarbons referred to and hot air which thus even permits reduction of the silica (SiO<sub>2</sub>).

It presents two zones, the one B a reducing zone in which eventually there takes place the commencement of fusion, which is fed with gases rich in carbon monoxide (CO) and in hydrogen whilst a surplus of combustible liquid is injected in relation to the amount of hot air supplied, and another zone C (a more or less oxidizing zone), in which the fusion takes place, which fusion is brought about by reducing the amount of combustible liquid in relation to the amount of hot air supplied so that carbon dioxide (CO<sub>2</sub>) is freed.

The furnace is provided with a chamber Z into which additions (of charge) are made, and which is heated by the hot gases produced in the oxidizing zone, by injection of hydrocarbons by tuyères S (Fig. 4). Into this chamber may be introduced powdered materials, and manganese ore to eliminate the last eventual traces of sulphur, these additions being kept in the chamber by the pressure of the gases issuing from the furnace.

The hot air is obtained by the combustion of gases leaving the furnace, collected in a circular conduit D (Figs. 4 and 5) and sent by a conduit G into alternative recuperator heaters situated adjacent the furnace, fitted with baffles N (Fig. 1) these gases being ignited by the heaters H. The hot air, driven by suitable ventilator means, passes through tubes I and K into circular conduits E and F surrounding the zones, and penetrates by tuyères S, spaced around the zones, into the latter.

The combustible liquid in a reservoir V (Fig.

1) being the light hydrocarbons free from sulphur, obtained in the first stage situated in a hot place of the furnace, is distributed by piping Q and R and is introduced into the furnace by 5 the same hot air tuyères already mentioned.

The furnace is cooled by means of water from a reservoir W, passing through a system of pipes situated in the actual masonry of the furnace, and provided with valves necessary to cause circulation of the water into the overheated parts, indicated by an escape of steam the purpose of which is to draw attention to the fact that the injection of combustible material on the side of the furnace opposite the overheated part 10 should be reduced.

The furnace is provided with an interior lining which takes part in the reactions and gives rise to the production of abundant slag which flows continuously to the furnace chamber. They are 15 collected in trough X filled with water and may be used as an agglomerant having the nature of cement.

It will be understood that the process may also serve for the treatment of manganese, chromium, 20 or other similar ores, and that the furnace may also be used in other metallurgical processes without departing from the scope of the invention.

What I claim is:

30 1. A two stage process for the production of cast-iron or steel, comprising subjecting in the first stage crude iron ores, crude solid carbonaceous distillable combustible materials and heavy liquid hydrocarbons or tars, to a heat treatment 35 at a temperature not greater than 500° C., to produce purified, agglomerated, carburized and partially reduced ore, high quality metallurgical coke and light liquid hydrocarbons, and subjecting said three products in a second stage, to heat treatment at temperatures ranging from 1000° to 2000° C., for the production, in a single fusion 40 operation, of cast-iron or steel.

2. A two stage process for the production of cast-iron or steel, comprising subjecting in the first stage iron ores, solid carbonaceous, distillable combustible materials and heavy liquid hydrocarbons, all of which may contain sulphur, 45 together to heat treatment, at atmospheric pressure in a retort at a temperature not greater than 500° C. and subjecting the three products so obtained in a second stage to a second heat treatment in a shaft furnace at a temperature between 1000° and 2000° C., for the production in a single fusion operation of cast-iron or steel.

55 3. In a two stage process for the production of cast-iron or steel, the step of producing charging products by subjecting together iron ores, solid carbonaceous combustible material and heavy hydrocarbons to heat treatment at 60 relatively low temperature, to distil the combustible materials, to crack the hydrocarbons and to reduce the ores, whereby there are obtained respectively agglomerated, carburized and partially reduced ore, metallurgical coke and synthetic light liquid hydrocarbons, the step of admitting said ores and coke mixed with common fluxing agents, manganese ores and iron scrap to the heating chamber of a shaft furnace and subjecting said mixture to temperatures 65 between 1000° and 2000° C., obtained by injecting said light hydrocarbons and hot air in controllable proportions.

70 4. In a two stage process for the production of cast-iron or steel, the step of producing charging products by subjecting together iron

ores, solid carbonaceous combustible material and heavy hydrocarbons to heat treatment at relatively low temperature to distill the combustible materials, to crack the hydrocarbons and to reduce the ores, whereby there are obtained respectively agglomerated, carburized and partially reduced ore, metallurgical coke and synthetic light liquid hydrocarbons, admitting said ores and coke mixed with common fluxing agents, manganese ores and iron scrap, to the 10 heating chamber of a shaft furnace, heating the upper zone of said furnace to a temperature of about 1000° C. by the injection of hot air and liquid hydrocarbons in controllable proportions to obtain a reducing zone and heating the lower 15 zone of said furnace also by injecting hot air and liquid hydrocarbons in controllable proportions to obtain an oxidizing and melting zone at a temperature of about 2000° C. whereby there is obtained cast-iron or steel as required. 20

5. A two-stage process for the production of cast-iron or steel, comprising subjecting in the first stage crude iron ores, crude solid carbonaceous distillable combustible materials, such as wood, lignite, coal and the like and heavy liquid 25 hydrocarbon residues or tars, together to a heat treatment at a temperature not greater than 500° C., to produce purified, agglomerated, carburized and partially reduced ore, high quality 30 metallurgical coke and light liquid hydrocarbons, and subjecting said three products in a second stage, to heat treatment at temperatures ranging from 1000° to 2000° C., for the production, in a single fusion operation, of cast-iron or steel. 35

6. A two-stage process for the production of cast-iron or steel, comprising subjecting in the first stage crude iron ores containing manganese, crude solid carbonaceous distillable combustible materials, and heavy liquid hydrocarbons, all of which may contain sulphur, together to heat 40 treatment, at atmospheric pressure in a retort at a temperature not greater than 500° C. and subjecting the three products so obtained in a second stage to a second heat treatment in a shaft furnace at a temperature between 1000° 45 and 2000° C., for the production in a single fusion operation of cast-iron or steel.

7. In a two-stage process for the production of cast-iron or steel the step of producing charging products by subjecting together iron ores, solid carbonaceous combustible material and heavy hydrocarbons to heat treatment at relatively low temperature to distil the combustible materials, crack the hydrocarbons and reduce the ores for the production respectively of agglomerated carburized and partially reduced ore, metallurgical coke and synthetic light liquid hydrocarbons; admitting said ores and coke in a second stage mixed with common fluxing agents, manganese ores and iron scrap to the 50 heating chamber of a shaft furnace, subjecting said mixture to a temperature between 1000 and 2000° C. obtained by injecting said light hydrocarbons and hot air in controllable proportions to produce cast-iron or steel and admitting the molten cast-iron or steel and slag to a reaction chamber adjacent said furnace at the base thereof and heated by gases from the lower zone of the furnace, adding in said chamber during operation powdered substances for the 55 removal of the last traces of sulphur and other materials according to the kind of cast-iron or steel required.

8. In a two-stage process for the production of cast-iron or steel the step of producing charg- 75

ing products by subjecting together iron ores, solid carbonaceous combustible material and heavy hydrocarbons to heat treatment at relatively low temperature to distil the combustible materials, crack the hydrocarbons and reduce the ores for the production respectively of agglomerated carburized and partially reduced ore, metallurgical coke and synthetic light liquid hydrocarbons; admitting said ores and coke in a second stage mixed with common fluxing agents, manganese ores and iron scrap to the heating chamber of a shaft furnace, subjecting said mixture to a temperature between 1000 and 2000° C. obtained by injecting said light hydrocarbons and hot air in controllable proportions to produce cast-iron or steel and adding during operation powdered substances for regulating oxidation according to the kind of cast-iron or steel required.

9. In a two stage process for the production of cast-iron or steel the step of producing charging products by subjecting together iron ores, solid carbonaceous combustible material and heavy hydrocarbons to heat treatment at relatively low temperature to distil the combustible material, crack the hydrocarbons and reduce the

ores for the production respectively of agglomerated, carburized, and partially reduced ores, metallurgical coke, and synthetic light liquid hydrocarbons, admitting said ores and coke mixed with common fluxing agents, manganese ores and iron scrap to the heating chamber of a shaft furnace having a thick lining, subjecting said mixture to temperatures between 1000° and 2000° C. obtained by injecting said light liquid hydrocarbons with hot air in controllable proportions, admitting the molten cast-iron or steel and slag to a reaction chamber adjacent said shaft furnace and at the base thereof and heated by gases from the lower zone of the furnace, adding in said chamber during operation powdered substances for the removal of the last traces of sulphur and other materials according to the kind of cast-iron or steel required, said additions being retained in the reaction chamber by the pressure of said gases, providing a system of conduits located in the masonry of the furnace through which water is circulated in controllable amounts to regulate the temperature of the masonry and of the lining of the furnace which is melted down in the reaction.

CONSTANTIN PAUL BRATASIANU.